

July 7, 1964

N. J. GRANT

3,139,682

STRENGTH RECOVERY OF DISPERSION HARDENED ALLOYS

Filed June 24, 1960



F/G. 1



F/G. 2

INVENTOR  
NICHOLAS J. GRANT  
BY  
E. J. Kail  
AGENT

3,139,682

STRENGTH RECOVERY OF DISPERSION  
HARDENED ALLOYSNicholas J. Grant, 10 Leslie Road, Winchester, Mass.  
Filed June 24, 1960, Ser. No. 38,521  
1 Claim. (Cl. 29—552.2)

This invention relates to a method for the recovery of high temperature properties of certain wrought metal compositions of the class based on the metal-metal oxide system in which a matrix metal or alloy has distributed therethrough a fine dispersion of a hard particle or refractory oxide phase.

In particular the invention is directed to the treatment of the aforementioned class of wrought metals which have been subjected to the deleterious effects of elevated temperatures wherein the physical and other properties of said metals have been substantially impaired. My invention is applicable to the recovery of those metals of the aforementioned class which have been impaired by heating to very high temperatures up to below the melting point of the matrix metal wherein recovery and softening has occurred; to those metals which have been subjected to brazing or solid state welding in which the properties at the braze or weld have been deleteriously affected; to those metals which have been heated to above the transformation temperature during fabrication or other treatments in which there has been a dissipation of stored energy with a consequent loss in strength; and to other situations in which prevailing high temperatures have had an adverse effect upon the physical properties of the metal.

Mechanical working, such as cold working, is known to increase the hardness and strength of conventional metals and alloys and it is not uncommon to provide commercially metals having varying degrees of strain hardening depending upon the ultimate use to which the metals are to be put. Generally, strain hardened metals, particularly metals incapable of being heat treated to higher hardnesses, are limited to room temperature applications or to temperatures not too far above room temperature for the reason that metals which have been strain hardened by cold working are not stable, but tend to revert to the strain free state when heated to temperatures which produce a softening effect on metals.

When a metal is subjected to cold working and thereafter heated to successively higher temperatures until softening sets in, the temperature at which this occurs is referred to as the temperature of recrystallization. The temperature of softening is related to the degree of strain hardening, that is the higher the amount of cold working, the lower is the temperature of softening or recrystallization. For example, a copper composition cold worked 3% (i.e. reduction by cold rolling) may exhibit a temperature of softening in the neighborhood of about 450° C. while the same composition cold rolled to a reduction of 20% may have a lower temperature of softening of about 400° C. At 50% cold work, the softening temperature may be about 350° C. while at 95% cold work, the temperature may fall below 300° C.

Because of the foregoing limitations, it has not been possible to utilize effectively mechanical working as a means of recovering physical or other properties of metals or alloys which have been impaired through overheating.

However, I have found that as to certain metal compositions, I can employ mechanical working, i.e. strain hardening, not only to recover properties lost through overheating, but in many instances to improve upon the properties then existing in the metal. By mechanical working, I include cold working as well as any working at temperatures above room temperature at which deformational energy is stored in the worked metal.

I have found, for example, that if the metal was orig-

inally in a condition of optimum strength and this was lost through aggravated heating at a very high temperature, well above the normal recrystallization temperature of the base metal or because of overheating due to welding or brazing, I can bring the metal back to its optimum condition by strain hardening without the metal tending to revert back to the strain free state at elevated temperatures when the recrystallization temperature of the unsupported matrix is exceeded. In other words, the strain hardened metal of my invention retains its high strength properties on heating to relatively high temperature levels with little dissipation of the stored energy, even above temperatures at which comparable metals or alloys generally recrystallize and soften. Moreover, whereas in conventional metals, e.g. cold worked copper, the temperature of recrystallization decreases substantially with increase in cold work, the compositions with which I work do not appear to be so affected and are relatively stable at elevated temperatures over a range of applied cold work.

It is the object of the invention to provide a method of providing wrought metal articles in which applied cold work is utilized to recover the strength properties of the metal without affecting the stability of the metal in resisting recrystallization at elevated temperatures.

Another object is to provide a method whereby certain metal compositions which have been softened by brazing or welding, such as spot, seam, butt or flash welding, or other forms of overheating can be recovered by mechanical working, whereby the metal thereafter will resist recrystallization at exceedingly high temperatures and substantially retain its stored energy.

These and other objects will more clearly appear from the disclosure and the appended drawings, wherein:

FIG. 1 depicts graphically the improved rupture life obtained for a cold worked alloy comprising copper and silica; and

FIG. 2 is similar to FIG. 1 but exhibits the improved rupture life obtained for a cold worked alloy comprising copper and alumina.

I have found that a metal containing a substantially uniform dispersion of finely divided substantially insoluble refractory material, e.g. refractory oxide, and whose properties have been impaired by substantial overheating, can be physically processed to confer improved high temperature properties, e.g. resistance to creep, by mechanically working said metal. Unlike the mechanical working of conventional metals and alloys, I find that the mechanical working of my material does not affect adversely the recrystallization temperature but that, on the contrary, the material so processed resists recrystallization at elevated temperatures well above the normal recrystallization temperature of the matrix metal and approaching the melting point in the alloys dispersion strengthened to an optimum.

A metal in which the foregoing phenomenon has been observed is copper, which metal, I pointed out hereinbefore, is particularly unstable in the cold worked condition at elevated temperature. I have found that when this and other ductile matrix metals, e.g. Fe, Ni, Pt, Au, Ag, Al, Zn, Pb and other of the well known commercially wrought metals or alloys based on these metals, contain aluminum, silicon and other metals in the stable oxide form, they can be cold worked to improve their high temperature properties beyond those normally obtained without adversely affecting substantially the temperature of recrystallization. The presence of the dispersion hardener is obtained in several ways, for example, either by mechanically mixing a substantially inert oxide, e.g.  $Al_2O_3$ ,  $SiO_2$ ,  $ThO_2$ ,  $ZrO_2$  and the like, with matrix metal powder followed by consolidation of the mixture into a wrought shape, or by internal oxidation.

In producing the material by internal oxidation, a refractory oxide-forming metal, e.g. aluminum, is alloyed as a dilute solution with a matrix metal, such as copper, and the alloy in particulate form, e.g. minus 44 microns, subjected to an oxidation treatment adapted to selectively oxidize aluminum to a dispersion of  $\text{Al}_2\text{O}_3$ , followed by consolidation of the particles to a wrought shape.

In one embodiment of the invention, alloys employed in the study were based on  $\text{Cu}-\text{Al}_2\text{O}_3$  and  $\text{Cu}-\text{SiO}_2$  produced by utilizing the technique of internal oxidation disclosed in copending application Serial No. 25,100, filed April 27, 1960. Briefly, copper-base alloys containing up to 2 percent of Al or Si according to the compositions shown in Table I were vacuum melted, chill cast into approximately 1.25 inch round bars, homogenized, and reduced to small chips by milling. The chips were ball milled until the powder product passed through 20 mesh screen. Each batch of powder was internally oxidized at temperatures shown in Table I.

Table I

| Alloy No. | Wt. Percent Element | Vol. Percent Oxide                | Oxidation Temp., °C. | Oxide Particle Radius, Å. |
|-----------|---------------------|-----------------------------------|----------------------|---------------------------|
| 1.....    | 0.07 Si.....        | 0.6 $\text{SiO}_2$ .....          | 750                  | 350                       |
| 2.....    | 0.25 Si.....        | 2.1 $\text{SiO}_2$ .....          | 750                  | 260                       |
| 3.....    | 0.09 Al.....        | 0.4 $\text{Al}_2\text{O}_3$ ..... | 650                  | 100                       |
| 4.....    | 0.09 Al.....        | 0.4 $\text{Al}_2\text{O}_3$ ..... | 750                  | 150                       |
| 5.....    | 0.23 Al.....        | 1.1 $\text{Al}_2\text{O}_3$ ..... | 650                  | 65                        |

The method adapted for internal oxidation of the alloy powders involved the surface oxidation of the powders to form a surface coating rich in  $\text{Cu}_2\text{O}$  (and also containing some solute oxide) by heating a given amount of powder in a measured amount of oxygen at about 450° C. The oxygen from the surface oxide was then diffused into the sample by heating at the desired temperature, e.g. 650° C., under substantially inert conditions. This method was found adequate for obtaining up to about 12% by volume of solute oxide within the matrix metal.

As an example of one method employed in effecting the internal oxidation of the alloy powder, the surface oxidized powder, for example 450 grams, is sealed in a 1.5 inch diameter tube by flattening of the ends. The tube is placed in a large muffle furnace held at the desired temperature, e.g. 650° C. or 750° C. for a time, determined by pilot tests, sufficient to obtain a uniform dispersion of solute metal oxide in each of the matrix metal particles.

The internally oxidized matrix metal powder is thereafter hydrogen reduced at an elevated temperature, e.g. 450° C. for one hour, to rid the surface of each particle of copper oxide and then packed by vibration in a copper container of about 1.4 inch I.D. by 4.5 inch long to achieve a pack density of about 50%. The container is evacuated and sealed and made ready for direct extrusion.

Of course, it will be appreciated that the foregoing method is by way of illustration and that many variations of accomplishing the same result may be substituted. For example, the internal oxidation could also be achieved by treating the alloy powder at a low partial pressure of oxygen (e.g. subatmospheric pressure) at which copper does not readily oxidize and the solute metal oxidized by diffusion of the oxygen into the matrix metal powder. However, I prefer in carrying out my invention to utilize the first method described as I find that this method lends itself to ease of control and readily reproducible results.

After the internal oxidation treatment, the powders are cleaned by hydrogen reduction and then extruded as aforementioned at 760° C. using a ram speed of about 55 inches per minute to give an extrusion ratio of about 75

28 to 1. Rods of approximately 0.25 inch diameter by four feet in length were obtained from the alloys.

Alloy No. 1 was partially recrystallized in the as extruded condition, that is part of the grains making up the copper matrix metal were equiaxed, indicating that some softening had occurred during hot working by extrusion. After subjecting this alloy to aggravated heating at just below the melting point of copper, 10 hours at 1050° C., the matrix metal was 100% recrystallized. The metal was then cold worked 25% and subjected to a rupture life creep test comprising heating the alloy at various stresses at 450° C. until rupture occurs. The results of the test indicated that the alloy in the cold worked condition was markedly superior at 450° C. to the extruded material, to pure copper and to the fully recrystallized alloy (note FIG. 1).

Alloy No. 5, which contained 1.1 vol. percent  $\text{Al}_2\text{O}_3$ , and which was 51% recrystallized by heating for 10 hours at 1050° C., was cold worked 10% and then subjected to a rupture life creep test as above. The results here indicated that the cold worked material had improved high temperature strength properties over the partially recrystallized condition and maintained these properties for prolonged periods of time at 450° C. without further recrystallization occurring. It will be noted from FIG. 2 that the material cold worked 10% exhibited marked improvement at high temperatures over the partially recrystallized material. Similar trends were noted with respect to alloy Nos. 2, 3 and 4. It is thus apparent that strain hardening in this class of alloys does not lower the temperature of recrystallization as in the conventional alloys but that, on the contrary, the stored energy is retained at elevated temperatures.

Likewise, similar results were obtained on dispersion hardened material produced by the mechanical mixing of powders. In producing alloys by mechanical mixing as disclosed in copending application Serial No. 24,971, filed April 27, 1960, matrix copper powder about 1 micron in size is mixed separately with specified amounts of finely divided  $\text{SiO}_2$  or  $\text{Al}_2\text{O}_3$ , preferably of particle size ranging from about 30 to 150 times smaller than the matrix metal powder, e.g. 0.02 micron. Dry mixing is used by utilizing a Waring Blender at a speed of about 15,000 revolutions per minute. The mixing is carried out for about 15 minutes and then further mixed by spatulation on a sheet of clean paper for a few minutes, the procedure with the Blender and the subsequent spatulation being repeated about four times.

The blended powder mixture is thereafter subjected to a reducing treatment in dry hydrogen for a minimum of five hours at a temperature of about 430° C. to insure clean particle surfaces for subsequent consolidation of the mixture into wrought shapes. Each batch of the mixed powders is introduced into a rubber tube supported within a perforated steel canister about two inches in diameter, one end of the rubber tube being rubber stoppered at the start. After the powder is introduced, a second rubber stopper having in communication therewith a hypodermic needle is inserted, a vacuum connection being made through the needle to remove the air from within powder mass. After completion of evacuation, the needle is removed and the canister assembly subjected to hydrostatic pressure at about 30,000 p.s.i. to yield compacts 1.4 inches in diameter and 2.5 inches long.

The compacts are then subjected to sintering in dry hydrogen for a minimum of 10 hours at 830° C. After that, they are each canned by insertion in a pure copper container and welding vacuum tight followed by extrusion at an elevated temperature. The extrusion ratio used is about 16 to 1, although the ratio could have ranged from 12 to 1 to 30 to 1.

Shapes produced by the foregoing manner, in which at least some of the grains of the matrix metal are equiaxed, can be further improved by cold working, whereby the worked material is capable of withstanding high stresses

at elevated temperatures for prolonged periods of time without recrystallization or without substantially losing its cold work temper.

The foregoing concept is particularly applicable to the treatment of alloys in which the matrix metal is subject to phase transformation during hot working. For example, dispersion hardened iron containing about 8% by volume of  $\text{Al}_2\text{O}_3$  was produced by extruding in the austenitic temperature range, e.g. about 1900° C. The extruded product exhibited a 100 hour rupture strength at 1100° F. of about 11,000 p.s.i. However, after cold working the same composition about 25%, the 100 hour rupture stress at 1100° F. was raised from 11,000 p.s.i. to 14,000 p.s.i., an increase of over 27%, the alloy, as cold worked, exhibiting particular resistance to creep at elevated temperatures while resisting recrystallization.

It is apparent that the invention is applicable to a wide variety of dispersion strengthened ductile matrix metals, be they based on alloy matrices or pure metals capable of being deformed into a variety of shapes. The lower melting metals Mg, Zn, Cd, Al, In, Pb, Sn and their alloys containing oxide dispersoids may be so treated. The higher melting metals comprising the copper group metals (Cu, Ag, Au) and their alloys, the platinum group metals (Pt, Pd, Ru, Rh, Ir, etc.) and their alloys, the iron group metals (Fe, Ni, Co) and their alloys may also be treated and so on.

Examples of copper group alloys are: 95% copper and 5% zinc; 90% copper and 10% zinc; 60% copper and 40% zinc; 71% copper, 28% zinc and 1% tin; 65% copper, 17% zinc and 18% nickel; 90% silver and 10% copper; up to 15% nickel and the balance silver; 70% gold and the balance palladium; 69% gold, 25% silver and 6% platinum, etc.

Examples of iron group alloys include: certain steels; 64% iron and 36% nickel; 31% nickel, 4 to 6% cobalt, and the balance iron; 54% iron and 46% nickel; 99% nickel and the balance cobalt; 68% nickel and 32% copper, etc.

Examples of platinum group alloys are as follows: platinum-rhodium alloys containing up to 50% rhodium; platinum-iridium alloys containing up to 30% iridium; platinum-nickel containing up to 6 or 10% nickel; platinum-palladium-ruthenium containing 77% to 10% platinum, 13% to 88% palladium, and 10% to 2% ruthenium; alloys of palladium-ruthenium containing up to 8% ruthenium; 60% palladium and 40% silver, etc.

Examples of refractory oxides which may be used in producing dispersion hardened alloys in accordance with the invention are  $\text{SiO}_2$ ,  $\text{Al}_2\text{O}_3$ ,  $\text{MgO}$ ,  $\text{BeO}$ ,  $\text{ZrO}_2$ ,  $\text{TiO}_2$ ,  $\text{ThO}_2$  and oxides of the rare earth metal group, such as oxides of cerium, lanthanum, neodymium, etc. Such refractory oxides are characterized as having a melting point above the melting point of the matrix metal and generally above 1500° C. In addition, these oxides are characterized by a negative free energy of formation at about 25° C. of over 90,000 calories per gram atom of oxygen. For example  $\text{SiO}_2$  has a negative free energy of formation at 25° C. of about 96,200,  $\text{Al}_2\text{O}_3$  of about 125,590,  $\text{MgO}$  of about 136,130,  $\text{BeO}$  of about 139,000, etc.

The amounts of the disperse phase employed may preferably range from about 0.1 to 15 vol. percent, preferably from about 1 to 12 vol. percent, and more preferably from about 3 to 10 vol. percent of the alloy. Where the disperse phase is produced by internally oxidizing an alloy containing an element which oxidizes easily to form a stable refractory alloy, e.g. aluminum dissolved in a matrix metal comprising copper, I prefer that the amount of disperse phase formed in this way not exceed about 6 vol. percent and more preferably range from about 0.1 to 4 vol. percent. I also prefer that the particle size obtained by internal oxidation range from about 60 to 700 A. average diameter.

Broadly speaking, the particle size of the disperse phase should not exceed 0.3 micron and preferably should range

from about 0.01 to 0.1. Where the dispersion strengthened metal is produced by powder mixing, the metal powder should be larger than the oxide by 30 to 250 times and preferably 30 to 150 times larger.

The amount of working applied to dispersion hardened material will depend upon the relative softness of the alloy and the amount of disperse phase present. Generally, the amount of working will be inversely related to the vol. percent of disperse phase present, that is, the higher the amount of disperse phase, the lower will be the amount of cold work required to achieve the desired effect. The amount of cold work in terms of reduction in cross sectional area may range up to about 30% and generally from about 10 to 25%. The working may be achieved by cold drawing, cold rolling, cold swaging, shot peening, or other forms of working in which a metal is deformed beyond its elastic limit at room or above room temperature at which recrystallization does not normally occur.

With respect to shot peening, hammer peening, cold forging, and the like, I have found that my invention is particularly applicable to the recovery of high strength in metals containing a disperse phase wherein overheating due to brazing, welding or other aggravated high temperature treatment has resulted in softening of the matrix metal.

By peening the affected area, the strength can be brought back to its original value or even higher with the additional advantage of resisting recrystallization at elevated temperatures well above the normal recrystallization temperature of the matrix. Thus, it is possible to overcome any weakness developed in a structural element due to localized overheating merely by peening the affected area.

Although the present invention has been described in conjunction with preferred embodiments, it is to be understood that modifications and variations may be resorted to without departing from the spirit and scope of the invention as those skilled in the art will readily understand, such modifications and variations are considered to be within the purview and scope of the invention and the appended claim.

What is claimed is:

A method of fabricating a wrought metal product at elevated temperatures which tend to impair the physical properties of at least a portion of the metal product being fabricated, such as occurs in welding, and at fabrication temperatures in excess of the recovery and recrystallization temperature of the metal product which comprises, providing a metal product to be fabricated comprising a metal selected from the group consisting of Fe, Ni, Co, Fe-base, Ni-base and Co-base alloys; Cu, Ag, Au, Cu-base, Ag-base and Au-base alloys; Pt, Pd, Ru, Rh, Ir and Pt-base, Pd-base, Ru-base, Rh-base and Ir-base alloys; and Mg, Zn, Cd, Al, Pb, Sn and Mg-base, Zn-base, Cd-base, Al-base, Pb-base and Sn-base alloys, having dispersed substantially uniformly therethrough about 0.1 to 15 volume percent of a stable insoluble disperse refractory oxide phase characterized by a negative free energy of formation at about 25° C. of at least about 90,000 calories per gram atom of oxygen and a particle size not exceeding about 0.3 micron, fabricating at least a portion of said metal product containing said disperse refractory oxide phase at an elevated fabrication temperature which tends to impair the physical properties of said portion, and then subjecting said fabricated portion to strain hardening, the amount of strain hardening being inversely related to the volume of the disperse refractory oxide phase present, whereby at least said strain hardened portion is characterized by improved high temperature strength properties equal to or above the original properties prior to impairment thereof by high temperature heating.

## References Cited in the file of this patent

## UNITED STATES PATENTS

2,317,295 Nesbitt ..... Apr. 20, 1943  
 2,390,023 Wyche ..... Nov. 27, 1945  
 2,716,080 Schwarz ..... Aug. 23, 1955

2,972,529 Alexander et al. ..... Feb. 21, 1961  
 3,019,103 Alexander et al. ..... Jan. 30, 1962  
 3,026,200 Gregory ..... Mar. 20, 1962  
 3,070,439 Grant et al. ..... Dec. 25, 1962  
 3,070,440 Grant et al. ..... Dec. 25, 1962